

## UNITED STATES PATENT OFFICE

2,523,000

## CHROMIUM NICKEL STEELS

Jacques Marcel Defranoux, Albertville, France,  
assignor to Societe D'Electro-Chimie D'Electro-  
Metallurgie et des Acieries Electriques D'Ugine,  
Paris, France, a corporation of France

No Drawing. Application May 16, 1949, Serial  
No. 93,631. In France May 28, 1948

2 Claims. (Cl. 75—125)

1

The cold-forming and cold-working of stainless chromium-nickel steels are, though taking place mostly under comparatively satisfactory conditions, limited by the decomposition of the austenite caused by said cold-forming and cold-working. Said decomposition renders the metal hard and brittle; it is, more particularly, very difficult to subject these steels to the chequering and decorative striking operations.

Furthermore, the articles obtained by means of such steels have a color which is not very agreeable and which markedly differs from that of silver or silver-plated articles.

The present invention, which has for its main object to remedy said disadvantages consists in adding copper to the chromium-nickel steel, the proportion of so added copper being near the limit of solubility of copper in said steel but not higher than said limit.

Thus, the proportion of copper to be added is a function of the analysis of the steel. It varies according to the ratio Cr/Ni and is the higher, the higher said ratio itself. It is, therefore, of about: 1% for a steel containing 18% nickel and 8% chromium, 2% for a steel containing 12% nickel and 12% chromium, 4% for a steel containing 12% nickel and 18% chromium or 8% nickel and 18% chromium; said proportions are maximum proportions.

Steels are thus obtained which are capable of being used for jewelry, decoration and domestic uses and which can be formed and worked in the cold with much less difficulty than the steels used hitherto. They are, more particularly, comparatively easy to roll, draw, chase, dish or chequer. Furthermore, they have, after polishing, a color which is nearer that of silver or silver-plated metal than the color of the usual chromium-nickel steels.

The addition of copper takes place in the course of manufacture of the steel by any means such as, for example, an addition of metallic copper to the liquid steel bath.

The following is an example of the manner in which the invention may be carried into practice. A steel was made which contained

12% chromium, 12% nickel and 2% copper. Said steel could be rolled readily and in a perfect manner without any incident. The hot or cold forming of said steel, more particularly its drawing, chasing or chequering could be effected with a truly unusual easiness.

Through a cold rolling giving an elongation of 20% without any intermediary reheating a breaking strength was obtained which did not exceed 60–65 kg./mm.<sup>2</sup>.

By drawing and for a reduction of section of 40% a strength was obtained which did not exceed 88–90 kg./mm.<sup>2</sup> and for a reduction of section of 70% a strength which did not exceed 125–127 kg./mm.<sup>2</sup>.

Finally, a glazed sheet of 20/10 mm. gave on a standardized chasing test of the Erichsen type a load which did not exceed 6,000 kg.

The color of said steel was silver white while that of a similar steel without addition of copper was slightly blue.

What I claim is:

1. Stainless steel consisting essentially of about 18% nickel, about 8% chromium, about 1% copper, and iron.

2. An ornamental article having a silver white appearance made from cold worked and polished stainless steel consisting essentially of about 18% nickel, about 8% chromium, about 1% copper, and iron.

JACQUES MARCEL DEFRAZOUX.

## REFERENCES CITED

The following references are of record in the file of this patent:

## FOREIGN PATENTS

|         |               |               |
|---------|---------------|---------------|
| Number  | Country       | Date          |
| 437,592 | Great Britain | Oct. 23, 1935 |

## OTHER REFERENCES

Alloys of Iron and Chromium, High Chromium, vol. 2, pages 433 and 434. Edited by Kinzel and Franks. Published in 1940 by the McGraw-Hill Book Co., New York.